

June 10, 1924.

1,497,539

G. A. BONE

METHOD FOR PERMANENTLY AFFIXING LETTERING ON ENAMELED SURFACES

Filed March 29, 1924

*Fig. 1.*



VARNISH-CONTAINING ENAMELED SURFACE

*Fig. 2.*



*Fig. 3.*



*Fig. 4.*



Inventor

George A. Bone,

By John M. Spellman  
his Attorney

Patented June 10, 1924.

1,497,539

# UNITED STATES PATENT OFFICE.

GEORGE A. BONE, OF WACO, TEXAS.

## METHOD FOR PERMANENTLY AFFIXING LETTERING ON ENAMELED SURFACES.

Application filed March 29, 1924. Serial No. 703,002.

To all whom it may concern:

Be it known that I, GEORGE A. BONE, a citizen of the United States, residing at Waco, in the county of McLennan and State of Texas, have invented certain new and useful Improvements in Methods for Permanently Affixing Lettering on Enameled Surfaces, of which the following is a specification.

10 This invention relates to the application of letters, figures, designs, trade-marks and other data as well as color, by hand painting, stenciling and printing, to the hard and glossy surface of enameled water-proofed fabrics and the like, and the prime object of the invention is to obtain a permanent bond between the letters or other data and the enameled surface such as will withstand the effects of the weather, washing, 20 handling and general and even unusual wear and tear.

Because of the hard and glossy surface and the lack of porosity of enameled water-proofed fabrics and the like, letters, designs and the like when hand painted, stenciled or printed thereon adhere but slightly to such hard surface, and consequently the letters can be readily scratched, and therefore ordinary wear and tear, washing and the effects of the weather soon cause the letters to 30 peel off.

The most satisfactory manner of applying letters and the like of course is by printing due to the rapidity of printing operations, but matter printed on enameled surfaces is the least satisfactory. My invention enables the use of the printing press for applying the letters or other matter because of the subsequent treatment whereby I effect 40 a permanent bond between the letters and the enameled surface.

While my invention is of general application, an important specific use to which it may be put is in the application of names, 45 trade-marks and other data to covers for spare tires carried by automobiles.

In carrying out my invention I take any common or well known enameled water-proofed fabric, such for instance as is employed in the making of spare tire covers, and I apply the color thereto in any manner to produce letters, designs or the like or to produce a blank panel thereon, and then the material is permitted to stand until the 55 color has become thoroughly dried, after which the article is subjected to heat suf-

ficient to soften the enamel coating or surface, and then the material is permitted to cool at atmospheric temperature, when it will be found that the color has become 60 strongly bonded to the enameled surface and will effectually withstand scratching, washing, the effects of the weather as well as hard usage.

This strong bond which is brought about 65 by the heating of the enameled surface to softness is due to the presence of varnish in the enamel coating, which varnish becomes soft under the action of the heat and when it subsequently dries and hardens it 70 holds the color, such as ink, paint or the like to the enameled surface in what is in effect an integral and therefore a permanent bond. In other words the varnish becomes fused and thereby produces the integral bond between the color and the enamel coating. 75 While the varnish ordinarily present in the enameled coating is sufficient to produce an effective bond, I prefer to include a small amount of varnish in the color employed, 80 and thereby add to the strength of the bond by bonding the varnish of the enamel with the varnish of the color.

While heat may be applied to the enameled water-proofed material in any suitable 85 manner, I have found that a satisfactory way of applying the heat is to place the material upon a hot plate with the enameled surface of the material uppermost. The hot plate may be heated by gas burners or 90 other heating means located immediately below the plate. Just as soon as the enameled surface becomes softened to a sticky or tacky condition, which can easily be determined by touching the surface and which is 95 also readily observable to the eye, the material is removed from the hot plate and set aside to cool off and dry. Of course the sheets of material should not be piled one upon the other as they are removed from 100 the hot plate because the softened enamel surfaces would stick to the underside of the superimposed sheets of material.

From the foregoing description of my invention, it will now be understood that the 105 color may be applied by hand painting, stenciling or printing, and that while printing on enameled water-proofed fabrics or other materials has hitherto been commercially impossible because a printed character does not resist wear, the effects of the weather, etc., my invention makes is com- 110

mercially possible to print the matter and enables me to produce signs and the like made of enameled water-proofed material in large quantities and at small expense.

5 In addition to having made a new and useful method, it is quite apparent that the product of my method is also new and useful.

In the drawing,

10 Figure 1 is a plan view of a sign embodying the features of the present invention,

15 Figure 2 is a side elevation of a hot plate and illustrating the heat treatment step of the invention,

Figure 3 is an enlarged fragmentary sectional view of the sign before heating,

20 Figure 4 is a view similar to Figure 3 but showing the condition of the sign after heating.

In practicing my invention I take a sheet of flexible material 1 which may be a fabric, leather or other material which has already been provided with a varnish-containing water-proofed enamel surface 2. The finished surface of this material is highly glazed, and as hereinbefore stated, matter printed thereon or otherwise applied thereto does not withstand wear and the 25 effects of the weather because the nonporous condition of the finished surface does not permit of the ink or color penetrating the surface. Such material usually has a black surface, is a stock proposition, can be 30 bought in the open market, and the specific structure thereof and method of making the same forms no part of the present invention. The lettering or other indicia or 35 ornamental matter 3 is printed or otherwise applied directly to the surface of the material or, if desired the letters may be applied to a panel 4 of color previously applied to the surface of the material. When 40 the color has become dried the material is placed upon a suitable hot plate 5 heated in any desired manner, as by a gas burner 45 6. The sheet of material is of course placed upon the hot plate with the back of the material against the plate. The enameled 50 surface of the material becomes softened under the action of the heat applied under atmospheric conditions, and this softening of the enameled surface is readily discernible to the eye, and when this change 55 occurs the sheet of material is removed from the hot plate and is placed aside to cool and thereby permit the varnish in the enameled surface to harden and bond the color 4 and the lettering 3 to the enameled 60 surface. In Figure 3 of the drawings the color panel 4 and the lettering 3 have been clearly indicated in their condition before heating, while in Figure 4 these elements have been shown in the condition they as- 65 sume after heating, wherein it will be seen

that these elements are bonded into the enameled surface 2 and in fact become an integral part thereof. It will be readily understood why it is that the color, the lettering or ornamental designs effectually 70 withstand wear and the effects of the weather.

What I claim is:

1. The herein described method which consists in applying color to the varnish-containing enameled surface of water-proofed flexible material, then subjecting the material to heat sufficient to soften the enameled surface portion which has the color applied thereto, separating the source 75 of heat and the material as soon as the surface thereof becomes softened, and then permitting the softened surface portion to cool and harden, whereby the color will be bonded by the hardened varnish to the 80 enameled surface.

2. The herein described method which consists in applying color to the varnish-containing enameled surface of water-proofed fabric, then subjecting the fabric 85 to heat sufficient to soften the enameled surface portion which has the color applied thereto, separating the source of heat and the material as soon as the surface thereof becomes softened, and then permitting the 90 softened surface portion to cool and harden, whereby the color will be bonded by the hardened varnish to the enameled surface.

3. The herein described method which consists in applying color to the varnish-containing enameled surface of water-proofed material, then placing the material upon a hot plate with the enameled surface uppermost and permitting the material to 95 remain thereon until the enameled surface 100 has become soft, and then removing the material and permitting it to cool.

4. The herein described method which consists in printing upon the varnish-containing enameled surface of water-proofed material, then heating the material until the printed surface portion thereof becomes soft, separating the source of heat and the material as soon as the surface thereof becomes softened, and then permitting the 110 softened surface portion to cool and harden whereby the printed matter will be bonded by the hardened varnish to the enameled 115 surface.

5. The herein described method which consists in applying color to the varnish-containing enameled surface of water-proofed flexible material, then applying heat to the back of the material until the colored enameled surface portion has become soft, separating the source of heat and the material as soon as the surface thereof becomes softened, and then permitting the softened surface portion to cool 120 and harden, whereby the color will be 125 seen

bonded by the hardened varnish to the enameled surface.

6. The herein described method which consists in printing upon the varnish containing enameled surface of flexible water-proofed material, placing the back of the material against a hot plate until the enameled surface becomes soft, and then remov-

ing the material and permitting the enameled surface thereof to cool. 10

7. As a new article of manufacture, water-proofed fabric provided with a varnish containing enameled surface having indicia fused thereto.

GEORGE A. BONE.